

## UNITED STATES PATENT OFFICE

2,001,621

## TREATMENT OF ARTIFICIAL FIBROUS MATERIAL

Leon Lilienfeld, Vienna, Austria

No Drawing. Application September 26, 1928,  
Serial No. 308,589. In Great Britain November 21, 1927

19 Claims. (Cl. 8—20)

This invention relates to a process for the treatment of artificial fibers, and is based on my discovery that the extensibility and elasticity of artificial fibers may be increased by a considerable amount by treating the artificial fibers with an alkali solution and carbon disulphide.

The invention, which consists in a treatment of artificial fibers with these reagents, is applicable to artificial fibers, especially artificial silk, which consists of or contains cellulose or cellulose hydrate, for example, to viscose silk, cuprammonium silk and "nitrate" silk. In referring to "viscose silk" in this specification, I embrace any and all silk (or fibers, threads, etc.) made from viscose by the use of any of the precipitating agents known. The process is of especial technical importance in its application to artificial fibers (hereinafter called "flasticized" artificial fibers) which are distinguished by a high strength, for example to artificial fibers which can be made by spinning viscose in a spinning bath consisting of or containing a strong mineral acid, particularly strong sulphuric acid, as described for example in my U. S. patent applications 113,582 and 113,583 filed June 3, 1926 and 156,751 filed December 23, 1926, (which applications have now matured into Patents 1,820,811, 1,683,200 and 1,683,199 respectively, the latter reissued as No. 18,170).

It is inherent in the products of my copending cases here referred to, that they possess high dry and wet tenacities, for example a dry tenacity exceeding 2 grams per denier, and in many cases very much more than this figure. However an objection to these products is the fact that they have only a low degree of extensibility (usually not over 4 to 5% and in any observed case not substantially over 7%) and a low degree of elasticity, both in fact considerably lower than ordinary good grade viscose silk.

By a strong mineral acid, or strong sulphuric acid (as herein referred to) is to be understood a mineral acid, the mineral acid content, for instance the sulphuric acid content of which, corresponds with that of a sulphuric acid containing at least 50 per cent of  $H_2SO_4$ . The acid can also be stronger, e. g. 70%  $H_2SO_4$ , more or less, see above cases.

The artificial fiber may be treated with an alkali solution and with carbon disulphide simultaneously, or separately with these reagents, in either order. That is to say, the fiber may be treated first with an alkali solution and then with carbon disulphide, or first with carbon disulphide and then with an alkali solution, or it may be treated with a mixture of carbon disulphide and an alkali solution, which mixture may be an emulsion of carbon disulphide in the alkali solution.

It is of importance that the treatment with

alkali solution and carbon disulphide should be such that the artificial fibers are not subjected to xanthogenation in too great a degree, that is to say to such a degree that they would dissolve or swell to too great a degree, or disintegrate during the treatment. In order to avoid too intense a treatment, the duration of the action of the carbon disulphide in presence of alkali should be suitably selected, and should not be too prolonged, or the strength of the alkali solution should not be too high. The danger that the artificial fibers may undergo dissolution or excessive swelling is very slight if the fiber is first saturated with carbon disulphide and then treated with an alkali solution, or if the fiber is treated with a mixture, for example an emulsion, of carbon disulphide and alkali solution.

It is preferable to conduct the treatment in such a manner that the fibers are not subjected to tension, or are subjected only to moderate tension: if, however, considerable tension be applied during any part of the treatment, it is desirable that the tension should be relieved or diminished at some moment at which a subsequent shrinkage of the fiber still appears possible, preferably before the fiber leaves the alkali solution, or before washing out the alkali.

The artificial fibers may be subjected to the treatment in accordance with the invention whilst they are in the dry state, or whilst they are moist, or wet: thus the invention may, if desired, be introduced into the spinning process, in which case the treatment may be applied to the fibers which leave the spinning bath, or after they leave the bath (for instance water), or if any, in which the bobbins rotate, or after the washing operation.

Artificial fibers, and in particular fabrics consisting of or containing artificial threads, when treated in accordance with this invention, not only acquire an increased extensibility and elasticity, but their tendency towards creasing is much reduced and in some cases may be wholly or nearly wholly eliminated.

The invention is applicable not only to artificial fibers, for example artificial silk, as such (whether in the form of threads, yarn or skeins or cops, or in the form of warps) but also to artificial fibers (such as artificial silk or staple fiber) in the form of woven material. It is also applicable to fibers or fabrics consisting either wholly of artificial fibers (such as artificial silk, staple fiber, or artificial wool), or containing mixtures of artificial fibers and natural fibers, that is to say, to threads or fabrics containing besides an artificial fiber another fibrous material, such as cotton, natural wool or natural silk. It is to be understood that the expression "artificial fibers of regenerated cellulose" as used in this specification is intended to include for example,

artificial silk, artificial wool, artificial cotton, artificial hair or other kinds of artificial fiber, in any of the forms as aforesaid and of the kinds hereinbefore stated.

5 The following examples illustrate the invention:—

*Example 1*

Viscose silk made by the process described in application No. 156,751, (which involves the treatment of the freshly formed viscose silk with  $H_2SO_4$  of 50% strength, or more, or other acid of equivalent strength), in the form of dried finished (but if desired, unbleached) skeins, is 10 impregnated preferably at room temperature, with carbon disulphide without application of tension, for instance by passing it through a bath containing carbon disulphide, by immersing it in carbon disulphide, or by spraying it with 15 carbon disulphide. The carbon disulphide may be used in undiluted form, or in conjunction with a suitable diluent, such as benzene or the like.

The duration of the treatment with carbon disulphide may be selected as desired. Generally, the yarn absorbs the requisite quantity 20 of carbon disulphide even during a period of from a few seconds up to two minutes, so that a short impregnating treatment is as a rule sufficient. The yarn impregnated with carbon disulphide, if desired after separating the excess of 25 carbon disulphide by pressing, centrifuging or the like, is then introduced into a caustic soda solution of 18-20 per cent strength and preferably at a temperature of 15-18° C., and allowed 30 to remain in this solution for 1-5 minutes. After removal from this bath, the yarn is freed, if required, from excess of caustic soda solution by pressing, centrifuging or the like (say at room 35 temperature), and is then introduced into sulphuric acid of 5-10 per cent strength, or into any other precipitating bath known in the viscose industry, for example a solution of ammonium sulphate of 10-25 per cent strength, hydrochloric acid of 4 per cent strength, or the known Müller bath or the like. These treatments may be performed at room temperature. After the yarn has been allowed to remain in the precipitating bath for a short time, it is removed, then washed and finally dried.

40 The silk, which prior to the treatment above described, showed an extensibility of 4-5 per cent, shows after the treatment an extensibility of 13-18 per cent, whilst its elasticity, which was originally 3.5-4 per cent, is increased by the 45 treatment to 5-6 per cent. The lustre of the silk does not suffer or suffers only moderately 50 from the treatment.

*Example 2*

55 The procedure is as in the preceding example, with the exception that the viscose silk is treated in the wet state, that is to say, the treatment with carbon disulphide and alkali solution is applied to the artificial silk immediately after the washing operation (and without intermediate drying) which follows the spinning operation, or (if the fiber has been spun on bobbins), which follows the twisting operation.

70 *Example 3*

The procedure is as described in Example 1 or Example 2 with the modification that there is used a caustic soda solution of 10 per cent 75 strength, kept at a temperature of 0° to -5° C.

*Example 4*

The procedure is as described in Example 1, Example 2 or Example 3, with the modification that the artificial silk is washed with hot or cold water after the treatment with the caustic alkali solution and before it is introduced into the precipitating bath.

*Example 5*

Artificial silk in skeins, as used in the preceding 10 examples, is introduced, without applying tension, into an emulsion or mixture, made in known manner of carbon disulphide and caustic soda solution of 18 per cent strength (for example consisting of 10 parts by weight of carbon disulphide 15 and 90 parts by weight of the caustic alkali solution), and allowed to remain in this emulsion or mixture for 2 to 10 minutes whilst the temperature is maintained at 15-20° C.

The material is then treated with acids or the 20 setting baths of the viscose industry, in the manner prescribed in Example 1 for the treatment of the material after its removal from the alkali solution in that example.

*Example 6*

Artificial silk in skeins as used in the preceding 30 examples is introduced into a caustic soda solution of 18-20 per cent strength at a temperature of 15° C., allowed to remain in this solution for about 1-5 minutes, and is then removed and if desired freed from excess of the alkali solution by pressing or centrifuging. The material is then introduced into a bath containing 35 carbon disulphide or it is exposed to the vapor of carbon disulphide. The treatment with carbon disulphide is continued for 2 to 10 minutes, whereupon the material is finished in the manner prescribed in the preceding examples.

*Example 7*

Mode of operation as in Example 6, with the exception that the strength of the caustic soda solution is 5 per cent only.

The procedure described in the foregoing 45 examples may be varied, for instance, by using another agent capable of precipitating viscose for example steam, instead of the precipitating agents therein named, and by using ordinary viscose silk of any kind, or copper silk (i. e. silk made from cuprammonium solution of cellulose) or nitrate silk, instead of the viscose silk specified therein.

The treatment described in the foregoing 55 examples may also be applied to artificial silk whilst the latter is in the stretched condition, or whilst it is subjected merely to a moderate tension: care should, however, be taken to discontinue or diminish the tension before the material is removed from the alkali solution.

The procedure for the treatment of fabrics, or of yarn containing besides artificial silk another fibrous material, such as cotton, follow from the examples which have already been given.

In the appended claims, I use the term "successive" to mean that the two reagents are employed one after the other, and not as intending to imply that the treatment with alkali solution must come before the treatment with carbon disulphide. And in said claims I use the term "joint" to cover the use of the several materials referred to in said claims, whether they are used simultaneously or successively (in any desired order).

The expression "artificial cellulose fibers" is 75

intended to include all artificial fibers consisting of, or containing cellulose or cellulose hydrate, that is, artificial fibers made from viscose, for example viscose silk, artificial fibers made from 5 solution of cellulose in cuprammonia, for example cuprammonia silk and denitrated cellulose nitrate artificial fibers, for example "nitrate silk".

I claim:—

1. A process for increasing the extensibility 10 and contraction of artificial fibers of regenerated cellulose, wherein the artificial fibers are treated with an alkali solution and carbon disulphide in any order and permitting shrinkage of said material to occur.

15. 2. A process as referred to in claim 1, wherein the artificial fibers are treated in substantially unstretched condition.

3. A process as referred to in claim 1, wherein the artificial fibers are in a stretched condition 20 during only a portion of the treatment, but the stretching is at least partially relieved before the fibers leave the alkaline bath.

25. 4. A process as referred to in claim 1, applied to viscose silk which has been made by spinning viscose in a bath which contains mineral acid of a strength corresponding to at least 50% of sulphuric acid.

30. 5. A process for increasing the extensibility of artificial fibers of regenerated cellulose, which process comprises the step of subjecting the artificial fibers while not in a strongly stretched condition to the joint action of an alkali solution and carbon disulphide and permitting shrinking of the 35 said material to occur.

35. 6. A process for increasing the extensibility of artificial fibers of regenerated cellulose, which process comprises subjecting the artificial fibers to the joint action of an alkali solution and carbon disulphide and subjecting the fibers to tension 40 during a part only of the entire process which includes said treatment and subsequent washing of the fibers.

45. 7. A process of making artificial silk which comprises the steps of spinning viscose into a bath containing a mineral acid of a strength equivalent to not below 50% of actual sulphuric acid, and subjecting the spun silk to the joint action of an alkali solution and carbon disulphide and permitting shrinking of the said material to occur.

50. 8. A process of making artificial silk which comprises the steps of spinning viscose in a bath containing not substantially below 50% of sulphuric acid and subjecting the spun silk to the joint action of an alkali solution and carbon disulphide and permitting shrinking of the said material to occur.

55. 9. A process of making artificial silk which comprises the steps of spinning viscose and subjecting same to a bath containing not substantially below 50% of sulphuric acid and subjecting the spun silk to the joint action of an alkali solution and carbon disulphide and permitting shrinking of the said material to occur.

60. 10. A process of making artificial thread which comprises the steps of spinning viscose in a bath which consists of mineral acid having a strength equivalent to at least 50%  $H_2SO_4$ , and subjecting the spun thread to the joint action of an alkali solution and carbon disulphide without substantially stretching during the latter part of such treatment.

11. A process of making artificial silk which comprises the steps of spinning viscose in a bath which contains not below 50% of sulphuric acid and subjecting the spun silk to the joint action of an alkali solution and carbon disulphide without substantially stretching during the latter portion of the treatment with alkali solution and carbon disulphide. 5

12. A process of making artificial silk which comprises the steps of spinning viscose, subjecting same to action of a bath containing mineral acid in amount equivalent to at least 50% of  $H_2SO_4$ , and subjecting the silk to the successive action of an alkali solution and carbon disulphide in any desired order and permitting shrinking of the said material to occur. 10 15

13. A process of making artificial thread which comprises the steps of spinning viscose in a bath which consists of sulphuric acid of at least 50% strength, subjecting the thread to the joint action of an alkali solution and carbon disulphide and avoiding substantial stretching during the latter portion of the treatment with alkali solution and carbon disulphide. 20

14. A process of treating such artificial cellulosic fibers as have a dry tenacity exceeding 2 grams per denier and which in their untreated condition have a relatively low degree of extensibility, which comprises treating such artificial fibers with an alkali solution and carbon disulphide, such steps being in any desired order and permitting shrinking of the said material to occur, whereby the extensibility is increased. 25 30

15. A process of treating such artificial cellulosic fibers as have a dry tenacity exceeding 2 grams per denier and which in their untreated condition have an extensibility not substantially exceeding 7%, which comprises treating such artificial fibers with an alkali solution and carbon disulphide, such steps being in any desired order and permitting shrinking of the said material to occur, whereby the extensibility of the fibers is increased. 35 40

16. A process for increasing the extensibility of regenerated cellulose fibers having a dry tenacity over 2 grams per denier, wherein the artificial fibers are treated with an alkali solution and carbon disulphide in any order and permitting shrinking of the said material to occur. 45

17. A process for increasing the extensibility of regenerated cellulose fibers having a dry tenacity over 2 grams per denier, which process comprises the step of subjecting the artificial fibers to the joint action of an alkali solution and carbon disulphide and permitting shrinking of the 50 55 said material to occur.

18. A process for increasing the extensibility of regenerated cellulose fibers having a dry tenacity over 2 grams per denier, which process consists in subjecting the artificial fibers to the successive action of an alkali solution and carbon disulphide and permitting shrinking of the said material to occur. 60

19. A process for increasing the extensibility of regenerated cellulose fibers, wherein the artificial fibers are treated with an alkali solution and carbon disulphide in any order, the latter portion, at least, of said treatment being performed while said fibers are not being stretched. 65